

# UNITED STATES PATENT OFFICE.

JOHN BEATTIE, OF LEETE ISLAND, CONNECTICUT.

## BATTERY-ZINC.

1,027,169.

Specification of Letters Patent.

Patented May 21, 1912.

No Drawing.

Application filed June 17, 1911. Serial No. 638,749.

*To all whom it may concern:*

Be it known that I, JOHN BEATTIE, a citizen of the United States, residing at Leete Island, in the county of New Haven and 5 State of Connecticut, have invented certain new and useful Improvements in Battery-Zincs, of which the following is a full, clear, and exact description.

This invention relates to amalgamated 10 battery zincs, and more particularly to a process for manufacturing the same, and has for its object the production of amalgamated zincs adapted for use in galvanic batteries, and the like, which are substantially 15 free from deleterious matter, and which are, further, more highly electro-positive than amalgamated zincs as produced by processes heretofore in use. These and other objects of my invention will be hereinafter set forth 20 and more particularly pointed out in the appended claims.

In the United States Letters Patent No. 359,838, dated March 22, 1887, I disclosed a process for making battery zincs which involved the use of lead and arsenic. The 25 said process was found to be fairly efficacious and the zincs manufactured by means of the same were quite thoroughly amalgamated. There were present, however, in such zincs 30 certain impurities, necessitated by the process, which were objectionable, and I now disclose an improved process whereby amalgamated zincs may be produced which are not only substantially free from deleterious matter, but which are actually more highly electro-positive than even an amalgamated zinc comprising simply zinc and mercury.

In amalgamating mercury and zinc, it is highly desirable that the process be conducted 40 in such a manner that the mercury shall not be volatilized to any considerable degree before complete amalgamation thereof with the zinc has been brought about. In the present process this is preferably effected by first forming an amalgam of mercury and a 45 light metal such as sodium, which may be readily accomplished at a low heat; and the quantity of sodium, if that be the metal used, present in such amalgam need not be in excess of four per cent. This sodium-mercury amalgam may be then cast into sticks or blocks of determined size, the small 50 quantity of sodium present therein being sufficient to impart considerable tenacity to it when cold. If desired the application of heat to the sodium and mercury, when form-

ing the amalgam thereof, may be effected in a closed receptacle and in a non-oxidizing atmosphere in order to completely prevent any oxidation of the sodium or volatilization 60 of the mercury. This is not however absolutely essential if care be exercised in the heating operation. A determined quantity of zinc or spelter of good quality is then heated to fusion in a crucible or melting pot, 65 which latter should preferably be of some material not adapted to alloy with the zinc; since, for example, if the melting pot be of iron, such metal will combine with the zinc to form a thick sediment of zinc-iron alloy, 70 which settles to the bottom of the pot and thereby causes considerable waste. A relatively small quantity of the sodium-mercury amalgam is now added to the molten zinc to form an amalgam comprising from two to 75 four per cent. of mercury; the heat at which this second step of the operation is conducted being also relatively quite low.

While I have specified sodium as the preferred metal to be amalgamated with the 80 mercury in the first step of the operation, I do not wish to be limited to this particular metal since other electro-positive metals may be utilized; said metals, of course, having the like property of forming with mercury 85 a firm and solid amalgam when cold, which amalgam need have but a small percentage of such electro-positive metal present therein. The alkali metals appear to be best adapted for this purpose; and sodium, being 90 the cheapest of these metals, is preferred. In any event it is most desirable that the metal amalgamated with the mercury in the manner above described should be at least as highly electro-positive as zinc, if not more 95 so; so that as a result of its presence in the ultimate product the electro-positive characteristic of the entire metallic mass is fully as high, or even higher, than that of zinc. The lead which was referred to in my previous 100 patent did not possess this qualification, and was hence deleterious in that its presence tended to make the resultant product less highly electro-positive than zinc alone; while furthermore both the lead and the arsenic constituted impurities which were otherwise objectionable.

The process as herein described is somewhat simpler than that set forth in my said 110 patent, and the product resulting therefrom is also preferable. I described in my former Patent 466,820, an amalgam consisting of

zinc, mercury and magnesium, but the element to which the present application relates possesses advantages over that described in said patent, in that the alkali metal, sodium, for example, is more highly electro-positive than magnesium. It will also be observed that the present element is substantially homogeneous throughout by reason of its mode of preparation or manufacture.

Having described my invention, I claim:

1. A substantially homogeneous electro-positive element for batteries which comprises an amalgam of zinc, sodium and mercury.

2. A substantially homogeneous electro-positive element for batteries which comprises an amalgam of zinc, mercury and an alkali metal.

3. An electro-positive element for batteries, the surface and also the interior portions of which comprise an amalgam of zinc, mercury and a metal more highly electro-positive than magnesium.

In witness whereof, I subscribe my signature, in the presence of two witnesses.

JOHN BEATTIE.

Witnesses:

AQUILA H. HULL,  
ALFRED R. GRISWOLD.

---

Copies of this patent may be obtained for five cents each, by addressing the "Commissioner of Patents,  
Washington, D. C."

---